

Sept. 21, 1948.

C. FRONDEL

**2,449,844**

## QUARTZ OSCILLATOR PLATES

Filed Dec. 15, 1944



Fig. 1.



Fig. 2.

INVENTOR  
CLIFFORD FRONDEL

BY

BY  
Fannie Davis, Marvin Edwards  
ATTORNEYS

Patented Sept. 21, 1948

2,449,844

# UNITED STATES PATENT OFFICE

2,449,844

## QUARTZ OSCILLATOR PLATE

Clifford Frondel, Flushing, N. Y., assignor to  
Reeves-Ely Laboratories, Inc., New York, N. Y.,  
a corporation of New York

Application December 15, 1944, Serial No. 568,330

18 Claims. (Cl. 171—327)

1

This invention relates to quartz oscillator plates and has for its object certain improvements in the method of manufacturing oscillator plates made of quartz or equivalent material.

In the manufacture of so-called BT quartz oscillator plates, for example, automatic or semi-automatic machines are generally employed in the initial and intermediate states. The final finishing of the plates is, however, still largely a hand operation, the work being done by highly skilled operatives, usually called finishers. In finishing the plates, physical dimensions of the order of sub-millionths of an inch are involved. The finisher is usually provided with a frequency-checking device, a flat glass plate, fine abrasive, an etching solution, water, a brush, cleaning solutions, lint-free towels, a micrometer, an optical flat, a small square, etc.

The finisher receives the plates, sometimes called blanks, as they come from mechanical lapping machines, the plates having been cut to substantially proper length and width and usually brought close to, but less than, the desired oscillating frequency. In a plate desired to have a final frequency of, say, 8000.000 kc., the machine lapping or other pre-hand-finishing treatment is stopped when the plate is from roughly a few hundred cycles up to ten or more kilocycles under the final desired frequency. A preliminary frequency check is then made by comparing the frequency of the plate with that of a standard plate having a known frequency. This gives the finisher a general idea how much hand lapping the plate should be given. To reduce the plate to its proper thickness, and hence to increase its frequency, the finisher grinds the plate in a mixture of the abrasive and water on the flat glass plate, keeping the faces of the plate as flat and parallel as possible. The plate is next thoroughly cleaned and dried, after which its frequency is again tested. This is done by inserting the carefully cleaned plate in a holder, plugging the holder into an oscillator circuit and noting whether or not the plate has reached the desired oscillating frequency. The lapping of the major plane surfaces of the plates usually is accompanied by a lapping or beveling of the edges of the plates; this operation, by removing roughness and other imperfections from the edges and by altering the edge dimensions, gives the desired degree of activity, so-called, to the plate.

The finishing of a plate to its desired frequency also may be accomplished in other ways, and a number of techniques other than hand lapping have been and are being developed in the oscillator-plate industry. Thus, in the so-called acid-

2

dip or etching process, the plates as obtained at the completion of the machine lapping are brought up to the desired frequency by dipping them for the required length of time into a solvent for quartz. This solvent, which may be, for example, hydrofluoric acid, removes quartz from the surface of the plate and thus acts to reduce the thickness of the plate to the desired value. This process, as with hand lapping, requires an intermittent, successive, series of treatments and measurements, especially in the final stages, to ensure that the desired frequency is exactly attained. The rate of etching of different plates of the same initial frequency is not identical, due to variations in the cleanliness of the surface, the roughness of the surface, and other factors, so that a uniform, timed, procedure for all plates can not be set out. In still another method of finishing plates to the desired frequency, the plates are tumbled with an amount of coarse abrasive in a container until the frequency approaches that desired. The plates are then removed, cleaned, and are adjusted to the desired frequency either by etching or hand lapping.

25 Alternate hand lapping, cleaning and testing are required until the plate reaches the desired frequency. The activity of the plate is determined by its dimensions, contour, parallelism, absence of flaws, cleanliness, etc. These physical characteristics are checked, changed, and rechecked until the desired activity is obtained. The frequency of the plate changes with changes made to the plate to obtain the desired activity, so that the finisher must coordinate the numerous variables going into the finishing operation to obtain a combination of conditions that yields a plate of predetermined activity and frequency.

30 Hand finishing by these methods of the oscillator plates is a tedious, slow, delicate and costly operation at best and leaves much to be desired. The human factor is an exceedingly important element in these finishing operations and the results obtained tend naturally to vary from person to person, depending upon the particular technique employed at the time by each finisher.

35 As a result of my investigation I have discovered that the frequency and certain other characteristics of piezo-electric bodies may be adjusted or varied without altering the physical dimensions 40 of the body, such as by grinding, etching or plating with a metal or other material. The frequency of oscillation of quartz oscillator plates, for example, may be varied continuously and this variation may be brought under continuous visual control as by an appropriate meter. This permits the frequency to be adjusted exactly to a pre-

determined value or range merely by following the frequency variation on a meter and stopping the treatment at the desired value or within the desired range. This is not possible in present methods of manufacture of piezo-electric bodies which, as noted above, involve a discontinuous alternating process of grinding or etching, cleaning and testing. The frequency of oscillation of quartz oscillator plates may, for example, be readily adjusted to a desired value with an accuracy up to 1 cycle or greater, depending primarily on the accuracy of the measuring device employed. This accuracy cannot be accomplished by the conventional method of grinding or etching because the amount of grinding or etching on which the change of frequency and accuracy depends cannot be accurately controlled or measured, and the change in frequency itself cannot be observed continuously.

The frequency of a piezo-electric body that has been put into a relatively stable state by means of baking, sulfuric acid washing or other treatment, such as for the purpose of eliminating or reducing spontaneous variation with time in the frequency or activity of the piezo-electric body, can be adjusted without destroying the stability of the piezo-electric body. This is not possible by present methods of manufacture. For example, if a number of quartz oscillator plates are brought by grinding or etching to a desired frequency, and are then baked or otherwise treated, for the purpose of stabilization, it is found that the frequency often changes erratically from the original value and must then be adjusted by additional grinding or etching. This action then destroys the stability of the oscillator plate and the purpose of the original stabilizing operation is lost. This readjustment can now be accomplished without grinding or etching and without loss of stability.

The frequency of oscillator plates may be adjusted, for example, without wetting them with water or other liquids and in an entirely dry condition. Water is commonly used in the conventional method of finishing to frequency by lapping with an abrasive or by etching, and has been considered to contribute substantially to undesirable ageing and other phenomena in the finished oscillator plate. This difficulty may now be obviated.

The initial change in frequency is downwards from the initial value and is brought about by treating the oscillator plates with radiant energy suitable for that purpose. This may be done, for example, in accordance with the inventions disclosed in my co-pending applications Serial Nos. 568,323, 568,324, now Patent Number 2,437,-912, 568,325, 568,326, now Patent Number 2,437,-913, 568,327, 568,328, now Patent Number 2,437,-914, and 568,329, now Patent Number 2,437,915, filed December 15, 1944; but the downward change is reversed and the frequency restored to its original or intermediate value by suitable treatment in accordance with the present invention. The new technique is especially advantageous in the recovery of oscillator plates that have been overshot by the ordinary methods of hand finishing. Oscillator plates that have increased in frequency over the upper tolerance due to ageing, or aged low activity plates that have gone over the tolerance after cleaning to bring up the activity, may be similarly readjusted to their original frequency.

In accordance with the invention, quartz oscillator plates that have been treated to the ac-

tion of a form of radiant energy adapted to decrease their oscillating frequency are subjected to the action of ultra-violet light rays in amount sufficient to increase their oscillating characteristics to a predetermined value or range.

The kinds of energy that are effective to decrease the oscillating frequencies of the oscillator plates include radiations of the wave type, such as X-rays and gamma rays; and radiations consisting of material particles, such as cathode rays or electrons, beta particles or fast electrons, alpha particles and deuterons, as more particularly described in said co-pending applications. The change is progressive and continues during irradiation but finally reaches a limiting value, determined by factors within the quartz, beyond which there is no further change. The rate of change appears to depend primarily on the kind and intensity of the radiation, but in part on variations in the properties of the quartz from specimen to specimen and on pre-treatment of the quartz. The continuity of the change is of great importance from a manufacturing point of view. The downward direction of the change is also of particular advantage.

The downward change in frequency brought about by the radiations is permanent under ordinary conditions, but can be reversed and the oscillator plate brought back to its original frequency by baking at a suitably elevated temperature or by irradiating the plate with ultra-violet rays. Ultra-violet rays reverse the action of the other types of radiation. The ability to reverse the downward change is a great advantage. In other words, the oscillator plates may be adjusted downwards and upwards in frequency repeatedly by the proper treatment.

The rate at which the downward change in frequency of the oscillator plates can be effected and the total amount of change is influenced by 40 the temperature at which the quartz is held during irradiation, and by previously baking the quartz at a suitably elevated temperature.

These and other features of the invention will 45 be better understood by referring to the accompanying drawing, taken in conjunction with the following description, in which:

Fig. 1 is a diagrammatic cross-sectional representation of an ultra-violet ray lamp showing a 50 quartz oscillator plate positioned before a window for treatment with ultra-violet rays; and

Fig. 2 is a similar diagrammatic cross-sectional representation showing a quartz oscillator plate 55 mounted in a holder connected to a frequency meter.

Referring first to Fig. 1, the apparatus shown comprises an evacuated quartz tube 10 having mounted therein a tungsten filament 11 at one end and containing a suitable amount of mercury 12. An anode is indicated at 9. The tube is surrounded by a protective housing 13 provided with a plurality of windows 14, 14'. A quartz oscillator plate 15 is shown in front of window 14, the plate being held on a sliding holder 16 movable in an upper track 17 and a lower track 18 by means of a handle 19. A stack of plates 15', 15'', 15''', etc., is shown in front of window 14'.

Referring next to Fig. 2, the apparatus shown 70 comprises a similar evacuated quartz tube 10 with a quartz oscillator plate 15 located in front of window 14 of casing 13. In this case, however, the oscillator plate is mounted in a holder 20.

The casing of the holder around the oscillator 75 plate is shown broken away in part to expose the

oscillator plate directly to the ultra-violet light rays. The holder is, in turn, connected with a frequency meter 21 by means of a pair of leads 22 and 23. The frequency meter may be of conventional design, having a needle 24 adapted to move back and forth over a graduated frequency scale 25, preferably divided to indicate cycles per second.

In the case of Fig. 1, when an arc is struck across the tube, the interior of tube 10 is gradually heated to a temperature sufficiently high to vaporize or boil mercury 12, so that the tube becomes filled with mercury vapor. The resulting ultra-violet light rays 26 pass through tube 10 and window 14 onto oscillator plate 15, as well as through window 14' onto oscillator plates 15', 15'', etc. The effect of the ultra-violet rays on each oscillator plate is gradually to increase its oscillating characteristics or frequency. The bombardment of the oscillator plate with the ultra-violet rays may be conducted until the oscillating characteristics or frequency of each oscillator plate falls within a predetermined range or value. In the case of the stack of plates 15', 15'', 15''', the plate nearest window 14' receives the greatest effect from the radiations, although the next succeeding plates are affected less and less progressively by the radiations. Plate 15 may be removed from window 14 by pulling slide 16 by means of handle 18.

In using apparatus such as that disclosed in Fig. 2, the desired frequency range or value may be noted visually on frequency meter 21. When needle 24 is deflected until it points at the desired frequency indicated by scale 25, the oscillator plate is taken out of the path of ultra-violet rays or the source of rays is shut off.

The change in frequency caused by the ultra-violet rays is upwardly. Oscillator plates irradiated as described in my co-pending applications, in order to increase their frequency, may be reverted in frequency to their initial or intermediate value when exposed to ultra-violet rays in the manner indicated. The change is accelerated by heating the quartz oscillator plates to 100-150° C. during irradiation with the ultra-violet rays.

The use of ultra-violet rays offers an important advantage. If for some reason the frequency of an oscillator plate should be decreased too much by the other types of radiation disclosed, its frequency may be increased to the desired value.

It will be clear to those skilled in this art that the invention lends itself to numerous modifications. It is possible, for example, to adjust the plate to a desired frequency at a given temperature by irradiating the plate, and bringing it to frequency, while it is held at that temperature in a suitable heating or cooling contrivance. This is not easily accomplished by the conventional lapping or etching techniques of finishing plates.

The rate of change of frequency of the plate during irradiation and also the total amount of frequency change that can be obtained (saturation value) can be modified by baking the quartz plate at a suitable temperature before it is irradiated. Thus, baking the quartz plate at a suitably elevated temperature has been found to increase both the rate of change and the amount of change of frequency over that which would obtain if the plate had not been baked beforehand.

While the practice of the invention has been described with respect to piezo-electric material in the form of quartz, it will also be clear to those skilled in this art that the invention is applicable to the treatment of other piezo-electric

materials, such as Rochelle salts, tourmaline, tartrates, etc. The invention is applicable to the treatment of any useful piezo-electric material the frequency and oscillating characteristics of which are to be varied under controlled conditions.

The actual lowest limit of the complete spectrum, containing sufficient of the ultra-violet, as against the X-rays, to be successful for my present purpose are not known. Those waves of angstrom unit length from 1850 to 4000 appear best for my purpose. Fluorite is transparent to wave lengths as low as 1200 angstroms and lithium to about 1083. With vacuum spectographs having concave gratings, wave lengths as short as 40 angstroms have been photographed.

In this lower range there is of course overlapping of the ultra-violet rays and X-rays and the range of the latter is considered to reach about 400 angstroms. The ultra-violet band of wave lengths from 1850 to 4000 or from 1850 to the visible are completely successful for my purpose. At some place between the limits of 1850 and 400 angstroms the ultra-violet ceases to function for my purpose and no change is effected in the oscillator plates. For my present purpose I include in the term or expression "ultra-violet light rays" all such portions of the extreme ultra-violet band as function to bring about a frequency change upwardly in a piezoelectric material. Therefore the extreme low of this band with which I am concerned begins some place between 400 and 1850 angstroms and the included band extends up to 4000 angstroms. In addition to the quartz mercury lamp herein disclosed, I have used an iron arc and a Hanovia "short ultra-violet lamp" as my sources of ultra-violet radiation.

I claim:

1. In the manufacture of quartz oscillator plates that have been irradiated to decrease their frequency of oscillation, the improvement which comprises treating each oscillator plate with ultra-violet light rays adapted to increase its frequency of oscillation.
2. In the manufacture of quartz oscillator plates that have been irradiated to decrease their frequency of oscillation, the improvement which comprises treating each oscillator plate with ultra-violet light rays adapted to increase its frequency of oscillation, and terminating the treatment of the plate with said ultra-violet light rays when its frequency of oscillation reaches a predetermined value.
3. In the manufacture of quartz oscillator plates that have been irradiated to decrease their frequency of oscillation, the improvement which comprises treating each oscillator plate while mounted in a holder connected to a frequency meter with ultra-violet light rays adapted to increase the frequency of oscillation of the plate, and terminating the treatment of the plate with said ultra-violet light rays when its frequency of oscillation reaches a predetermined value.

4. In the manufacture of quartz oscillator plates that have been irradiated to decrease their frequency of oscillation, the improvement which comprises treating each plate while mounted in a holder connected to a frequency meter to the action of ultra-violet light rays adapted to pass through the housing of the holder and to increase the frequency of oscillation of the plate, and terminating the treatment of each plate with said ultra-violet light waves when its frequency of oscillation reaches a predetermined value.

5. In the manufacture of quartz oscillator

plates that have been irradiated to decrease their frequency of oscillation, the improvement which comprises maintaining each oscillator plate at a predetermined temperature, treating each plate at said temperature with ultra-violet light waves adapted to increase its frequency of oscillation, and terminating the treatment of each cooled plate with said ultra-violet light waves when its frequency of oscillation reaches a predetermined value.

8. In the manufacture of quartz oscillator plates that have been irradiated to decrease their frequency of oscillation, the improvement which comprises cooling each oscillator plate while mounted in a holder connected with a frequency meter, treating the plate while cooled with ultra-violet light waves adapted to increase the frequency of oscillation of the plate, and terminating the treatment of each cooled plate with said ultra-violet light waves when its frequency of oscillation reaches a predetermined value.

7. In the manufacture of quartz oscillator plates that have been irradiated to decrease their frequency of oscillation, the improvement which comprises maintaining each oscillator plate at a predetermined temperature while mounted in a holder connected with a frequency meter, treating each plate to the action of ultra-violet light waves adapted to increase the frequency of oscillation of the plate, and terminating the treatment of each plate with said ultra-violet light waves when its frequency of oscillation reaches a predetermined value.

8. In the manufacture of quartz oscillator plates that have been ground to a thickness beyond that required to increase its frequency to a predetermined value and that have then been irradiated to decrease their frequency of oscillation, the improvement which comprises treating each plate with ultra-violet light waves adapted to increase its frequency of oscillation.

9. In the manufacture of quartz oscillator plates that have been ground to a thickness beyond that required to increase its frequency to a predetermined value and that have then been irradiated to decrease their frequency of oscillation, the improvement which comprises treating each plate with ultra-violet light waves adapted to increase its frequency of oscillation, and terminating the treatment of each ground plate with said ultra-violet light waves when its frequency of oscillation reaches a predetermined value.

10. In the manufacture of quartz oscillator plates that have been ground to a thickness beyond that required to increase its frequency to a predetermined value and that have then been irradiated to decrease their frequency of oscillation, the improvement which comprises maintaining the plate at a predetermined temperature, treating the ground plate while at said temperature with ultra-violet light waves adapted to increase its frequency of oscillation, and terminating the treatment of each ground plate with said ultra-violet light waves when its frequency of oscillation reaches a predetermined value.

11. In the manufacture of quartz oscillator plates that have been etched to a thickness beyond that required to increase its frequency to a predetermined value and that have been irradiated to decrease their frequency of oscillation, the improvement which comprises treating each plate with ultra-violet light waves adapted to increase its frequency of oscillation, and terminating the treatment of each plate with said ultra-

violet light waves when its frequency of oscillation reaches a predetermined value.

12. In the manufacture of quartz oscillator plates that have been etched to a thickness beyond that required to increase its frequency to a predetermined value and that have been irradiated to decrease their frequency of oscillation, the improvement which comprises maintaining each plate at a predetermined temperature, treating each plate at said temperature with ultra-violet light waves adapted to increase its frequency of oscillation, and terminating the treatment of each plate with said ultra-violet light waves when its frequency of oscillation reaches a predetermined value.

13. In the manufacture of quartz oscillator plates that have been stabilized by baking, acid washing or other treatment, that have been irradiated to decrease their frequency of oscillation and that have a frequency of oscillation lower than desired, the improvement which comprises treating each oscillator plate with ultra-violet light waves adapted to increase its frequency of oscillation, and terminating the treatment of each plate with said ultra-violet light waves when its frequency of oscillation reaches a predetermined value.

14. In the manufacture of quartz oscillator plates that have been irradiated to decrease their frequency of oscillation, the improvement which comprises heating each plate to an elevated temperature to sensitize it to frequency change, treating each sensitized plate to the action of ultra-violet light rays adapted to increase its frequency of oscillation, and terminating the treatment of each plate with said ultra-violet light rays when its frequency of oscillation reaches a predetermined value.

15. In the manufacture of quartz oscillator plates that have been irradiated to decrease their frequency of oscillation, the improvement which comprises heating each plate to an elevated temperature to sensitize it to frequency change, treating each sensitized plate while mounted in a holder connected to a frequency meter to the action of ultra-violet light rays adapted to increase its frequency of oscillation, and terminating the treatment of each plate with said ultra-violet light rays when its frequency of oscillation reaches a predetermined value.

16. In the manufacture of quartz oscillator plates that have been irradiated to decrease their frequency of oscillation, the improvement which comprises treating such oscillator plates with ultra-violet light rays in the range from 1850 angstroms to 4000 angstroms to increase its frequency of oscillation.

17. In the manufacture of quartz oscillator plates that have been irradiated to decrease their frequency of oscillation, the improvement which comprises maintaining each oscillator plate at a predetermined temperature, treating each plate at said temperature with ultra-violet light rays in the range from 1850 angstroms to 4000 angstroms to increase its frequency of oscillation, and terminating the treatment of each cooled plate with said ultra-violet light rays when its frequency of oscillation reaches a predetermined value.

18. The method of increasing the frequency of oscillation of a piezoelectric oscillator comprising treating such oscillator with ultra-violet light rays in the range from 1850 angstroms to 4000 angstroms.